

## UNITED STATES PATENT OFFICE

2,218,973

## PRODUCING OF FREE-MACHINING STAINLESS STEEL HAVING A LOW SULPHUR CONTENT

Vincent T. Malcolm, Indian Orchard, Mass., assignor to The Chapman Valve Manufacturing Co., Indian Orchard, Mass., a corporation of Massachusetts

No Drawing. Application October 18, 1939,  
Serial No. 300,016

2 Claims. (Cl. 148—21.5)

This invention relates to improvements in producing a free-machining stainless steel of the ferritic type having a low sulphur content and is directed more particularly to the provision of a free-machining stainless steel having all the desirable characteristics inherent in steels of the same type which have a relatively high sulphur content but none of their disadvantages.

It has for some time been the practice to make stainless steels of the ferritic type for use in the manufacture of such machined parts as valve stems, other valve parts, etc., by means of such machines as so-called automatic screw machines which operate at high speeds, but success has only been had, as far as efficiency, speed, and economy are concerned, when these steels have had a sulphur content of approximately .25 to .50%. That is to say, stainless steels of the ferritic type having what is considered a relatively high sulphur content, that is between .25 to .50%, when operated upon in automatic screw machines give up chips which are cut or turned short and which are brittle so as to break away rapidly from the tool, with the result that the tool is kept clean and rapid, free cutting or turning is possible.

This, of course, is all as desired since the attainment of speedy efficiency is obviously the reason for the development and use of automatic machines.

However, the oil, chemical, and other industries which employ machined steel parts under such conditions that they are subjected to the action of various gases and acids at high temperatures have for some time objected to the corrosiveness and high degree of brittleness in such steels. That is to say, while stainless steels of the ferritic type having this relatively high sulphur content are capable of rapid and efficient machining, the sulphur content at the same time has been more or less of a contaminating element wherefore such steels are not satisfactory for use in these industries for the reasons stated.

Other stainless steels of the ferritic type containing relatively less sulphur have, of course, been produced but they are not readily adapted for machining in automatics. That is to say, stainless steels containing less than about .05% sulphur have been made but they have never been used with success in automatic machines which operate at high speeds since the cutting speed of such a low-sulphur-content stainless steel is about 30 feet per minute as contrasted with a cutting speed of around 100 feet per min-

ute of a stainless steel containing the larger amount of sulphur above mentioned.

Further, the outside threading and finishing of a stainless steel having a low sulphur content on an automatic high-speed machine is rough and of poor quality and tapping thereon is practically impossible. That is, such steels have had to be removed from the automatic machines and tapped and threaded by more or less of a hand method.

A further disadvantage of stainless steels of the ferritic type which have purposely been made with a relatively low sulphur content in order to satisfy the industries mentioned is that the life of the tools is shortened about 50% and re-grinding of the tools is necessary after working on five lengths of twelve feet as contrasted with every thirty such bars as previously. This, of course, is a serious objection and defeats the very purpose of high-speed automatic machining.

It is, accordingly, the principal object of this invention to provide a stainless steel of the ferritic type which does not have the corrosive or objectionably brittle qualities of such steels containing the relatively high amount of sulphur but which has their fine machining qualities. In other words, by the method of this invention, I take a stainless steel of the ferritic type having a low sulphur content and give to it the machining properties of a similar steel having a higher sulphur content while eliminating the contaminating influence thereof.

The formula of a common stainless steel of the ferritic type having a relatively high sulphur content and which has met with success as far as its machinability is concerned, is as follows:

|            | Percent                  |
|------------|--------------------------|
| Carbon     | maximum .15              |
| Manganese  | maximum .50              |
| Silicon    | maximum .50              |
| Phosphorus | maximum .04              |
| Nickel     | maximum .50              |
| Chromium   | maximum 11.5-13.0        |
| Sulphur    | approximately .25 to .50 |

As stated, however, such steels are not adapted for use in oil refineries, for example, where the machined valve stems or the like must withstand the action of acids and gases at elevated temperatures.

According to this invention, I employ a steel having the same approximate formula set forth above except that the sulphur content of the steel I work has a maximum sulphur content of .05%.

For the purposes of this invention, in the melting and pouring of the steel, I have found that it is desirable that both the proportions of the elements, and particularly the ratio of carbon and chromium, and the pouring temperature of the steel be such that the steel which results after a heat treatment about to be described contain not appreciably, if any, more than 10% of free ferrite. I also desire that any tendency towards "banding" or ferritic segregation be eliminated.

The method of the invention consists of a novel manner of treating the steel work with heat and, because of its nature, no subsequent tempering or drawing is required. As a first step, I preferably heat the steel to a temperature of from 1500° to 1600° F., and preferably to about 1550° F., and soak it a sufficient length of time until the heat penetration is complete.

20 The steel is then allowed to cool slowly with the furnace. As the next step I reheat the steel to a temperature within range of from 1550° to 1625° F.

25 The preferred reheating temperature is about 1580° F. and the steel is allowed to soak in this heat long enough for complete penetration. The final step consists in allowing the work to cool rapidly in air.

If desired, the first step may be eliminated.

30 That is the initial heating to between 1500° and 1600° F. and slow cooling may be omitted and the treatment confined to the heating to saturation at about 1580° F. and cooling rapidly in air.

Such a treatment, I have found, results in a 35 stainless ferritic steel of low sulphur content having a cutting speed in an automatic screw machine increased from 30 feet to 140 feet per minute. Further, steel processed according to this invention, notwithstanding the fact that it is of low sulphur content, has a tool-life 10 times greater than the tool-life of steels heretofore known.

40 It has also been found that with steels processed according to this invention, tapping, threading, and finishing may be efficiently done on automatic machines operating at high speed, thereby eliminating separate operations. Still further, the times of regrinds of tools operating on steels of this invention is increased about 400% and one automatic machine working thereon will do as much machining and more efficiently, as did three machines on steels of the previous practice.

45 Steels subjected to my special treatment developed all the desired physical properties such as tensile strength, impact value, etc., in a de-

gree equal to, if not superior to steels subjected to orthodox treatment.

It is also a fact that my method of treating low-sulphur-content steels such as I have described results in the same having a hardness of 5 from 280 to 340 Brinell.

The present well known method of heat treating stainless steels of the ferritic type, as described, has been to heat to a temperature of at least 1700° and quench in oil, then reheat to a 10 suitable temperature (known as drawing or the like) for the desired physical properties. This latter temperature may range between 400-1200° F. and while, by this treatment, Brinell hardness numbers of 220 to 360 may be obtained, the steel 15 is non-machinable in automatic screw machines.

In other words, the steels of this invention have the advantage of being considerably harder than most of those heretofore known but at the same time they are readily machinable and non-corrosive.

While I have described the invention in great detail and with respect to the present preferred form thereof, it is not desired to be limited thereto since changes and modifications may be made 25 therein without departing from the spirit and scope of the invention. The invention may be embodied in other specific forms without departing from the essential characteristics thereof. The present embodiments are therefore to 30 be considered in all respect as illustrative and not restrictive, the scope of the invention being indicated by the appended claims rather than by the foregoing description, and all changes which come within the meaning and range of equivalency of the claims are therefore intended to be 35 embraced therein.

What it is desired to claim and secure by Letters Patent of the United States is:

1. The steps in the process of producing free-machining ferritic stainless steel having less than .05% sulphur consisting of, heating the steel to a temperature within a range of from 1500° F. to 1600° F., allowing it to cool slowly, reheating the steel to a temperature within a range of from 1550° F. to 1625° F., and then cooling the steel rapidly in air. 40

2. The steps in the process of producing free-machining ferritic stainless steel having approximately .05% sulphur consisting of, heating the steel in a furnace to about 1550° F., allowing it to cool slowly within the furnace, reheating the steel to about 1580° F., and then cooling the steel rapidly in air. 45 50

VINCENT T. MALCOLM.

55